

## 1

2,964,176

PACKAGING CONTAINER AND PROCESS OF  
PACKAGING MATERIALS

Frank Herrmann, Lahr, Schwarzwald, Germany, assignor  
to Kunststoffwerk Lahr G.m.b.H., Lahr, Dinglingen,  
Schwarzwald, Germany

No Drawing. Filed Aug. 27, 1959, Ser. No. 836,319

Claims priority, application Germany Sept. 4, 1958

7 Claims. (Cl. 206—84)

The present invention relates to a packaging container for filling up and packaging solid, meltable products which are sticky when molten, and more particularly, to such a packaging container made from polypropylene and to a process of filling up and packaging such materials into said containers.

In several technical fields it is necessary to pour hot liquid materials, for instance bitumen or high melting point paraffins, for storage or shipping purposes into containers. Up to the present, such materials have generally been put into sheet metal containers. These sheet metal containers are stable. However, it is difficult to get the materials out of such containers again, as they adhere to the sheet metal even in the heated and molten state. For this reason, jute sacks impregnated with alginates and calcium chloride have also been used for packaging such materials. Packaging containers of this latter kind are, however, relatively expensive. Attempts have also been made to use plastics and paper for packaging such materials. However, many of these packaging materials are practically useless for this purpose because they are too sensitive to heat. On the other hand, the hot liquid materials which are to be packed are inclined to adhere to those plastics which are sufficiently heat-resistant.

Therefore, it is one object of the present invention to provide a packaging container for filling up and packaging solid, meltable products which are sticky when molten and which are to be packaged when hot, which container may readily be removed from the packaged material.

Another object of the present invention is to provide a process of filling up and packaging solid, meltable products which are sticky when molten and which are to be packaged when hot. Other objects of the present invention and advantageous features thereof will become apparent as the description proceeds.

It has been found that polypropylene is very well suited for packaging containers for materials which are to be packaged while hot. Unexpectedly, polypropylene does not consolidate with hot bitumen or paraffins and can be stripped from the cooled bitumen or paraffin without difficulty which fact is all the more surprising as polyethylene cannot be used for these purposes. For the purposes of the present invention, packaging containers, for instance bags of a suitable material such as paper bags, may be used, the inner surface of which is lined with polypropylene foils.

In the process according to the present invention the solid, meltable products which are sticky when hot and molten are filled up and packaged in containers of polypropylene, preferably polypropylene bags in the hot and molten state.

## 2

The packaging of the hot materials according to the present invention is preferably carried out in such manner that during the filling process the preformed container of polypropylene is supported in a correspondingly shaped rigid container, for example of metal sheet. If desired, a frame of a suitable material, for instance metal sheet or plastic, may be placed into the opening of the bag-like container in order to suspend it, reinforce its upper edge and keep it open while pouring the hot and liquid material to be packaged. After the hot material has been poured into the polypropylene container and has cooled, the frame-like reinforcement is removed and the filled polypropylene container is removed from the supporting container of metal sheet. When using propylene films or foils of wall thickness of from 0.03 to 0.05 mm. it is possible to package bitumen in this way in amounts of 30 kg. in weight for instance without difficulty.

According to another embodiment of this invention the polypropylene packaging containers are of various colours so as to distinguish different qualities of the packed material.

What I claim is:

1. Packaging containers for packaging solid, meltable products which are sticky when hot and molten, in the hot and molten state, said containers consisting of polypropylene.
2. Packaging containers for packaging solid, meltable products which are sticky when hot and molten, in the hot and molten state, said containers consisting of a polypropylene bag.
3. Process of filling up and packaging solid, meltable products which are sticky when hot and molten, the steps which comprise melting said products, pouring them into bags of polypropylene foils placed into a removable rigid correspondingly shaped container, cooling down the products, and removing the rigid container.
4. Process of filling up and packaging solid, meltable products which are sticky when hot and molten, the steps which comprise melting said products, pouring them into bags of polypropylene foils placed into a removable rigid correspondingly shaped container and suspended and reinforced at the opening by a rigid frame placed removably in the opening of the bag, cooling down said products, and removing the rigid frame and container.
5. A package of a solid meltable product which is sticky when hot and molten comprising said product and a container for said product, said container consisting of polypropylene foils.
6. A package of bitumen comprising bitumen and a container for the bitumen, said container consisting of polypropylene foils.
7. A package of high melting point paraffine comprising high melting point paraffine and a container for said high melting point paraffine, said container consisting of polypropylene foils.

## References Cited in the file of this patent

## UNITED STATES PATENTS

- |           |               |               |
|-----------|---------------|---------------|
| 2,348,622 | Heilman       | May 9, 1944   |
| 2,804,205 | Barton et al. | Aug. 27, 1957 |
| 2,834,768 | Friedlander   | May 13, 1958  |
| 2,840,551 | Field et al.  | June 24, 1958 |